

Patented Dec. 28, 1926.

1,612,679

# UNITED STATES PATENT OFFICE.

FERNANDO SOMOZA VIVAS, OF LOS ANGELES, CALIFORNIA.

## FIREPROOF SHELLAC.

No Drawing. Application filed November 11, 1924, Serial No. 749,293. Renewed May 26, 1926.

The invention relates to shellac and has as an object the provision of a dissolved gum of this nature which shall be fire proof instead of highly inflammable as is the shellac now in use.

An object of the invention is the provision of a shellac which while being fire proof shall not be unduly expensive to manufacture.

A further object of the invention is the provision of a fire proof shellac the qualities of which, for the purpose for which shellac is generally used, shall not be harmed by the ingredients which make it fire proof. The formula which it is preferred to use as a physical embodiment of the invention with the proportion of parts is as follows:

Parts.

|                      |     |
|----------------------|-----|
| Shellac              | 4   |
| Absolute alcohol     | 2   |
| Borax                | 1   |
| Perchlorethane       | .05 |
| Carbon tetrachloride | 2.5 |

Minor changes may be made in the proportion of parts or known equivalents for some of the ingredients named may be substituted therefor without departing from the spirit of the invention.

I claim as my invention:

1. A fireproof shellac comprising, in combination, gum lac, alcohol, borax, perchlorethane, and carbon tetrachloride, in proportions to provide a fireproof shellac. 30

2. A fireproof shellac, comprising, in combination, gum lac 4 parts, absolute alcohol 2 parts, borax 1 part, perchlorethane  $\frac{1}{2}$  part, 35 and carbon tetrachloride  $2\frac{1}{2}$  parts.

FERNANDO SOMOZA VIVAS.